

## UNITED STATES PATENT OFFICE

OLIVER B. HUSKEY, OF LOS ANGELES, CALIFORNIA

## IGNITION INSULATION COMPOSITION

No Drawing.

Application filed March 14, 1931. Serial No. 522,792.

This invention relates to improvements in compositions for use in protecting and insulating electric wiring and other electricity conducting bodies and is intended primarily, 5 for use in insulating the wiring system of the internal combustion engines of motor vehicles, airplanes, motor-boats, etc.

The primary object of the present invention is to provide a composition which may 10 be applied to the parts of an electric system while the same is wet, as well as when it is dry, and will operate immediately to insulate the parts and restore the previously shorted system to operative condition.

15 A still further object of the present invention is to provide a composition which may be readily spread over the wiring and other electrical parts of engines and which will adhere thereto and form thereover a protecting 20 coating or skin which will remain unaffected by rain water, salt water, or any of the usual atmospheric conditions which frequently operate to interfere with the proper performance of electric systems particularly 25 those systems used in airplanes, motor vehicles and the like.

The present composition is particularly 30 suitable for use on the ignition systems of airplane motors, especially the motors of hydro-planes.

It has been determined that the cause of a 35 great many airplane deaths has been stalling motors, due to the formation of vapor on the electric wires and inside of the distributor 40 heads, caused by sudden changes in atmospheric conditions. By the use of the present composition this vapor is prevented from forming electrical connections between the wires and other current carrying elements.

Another use to which the present composition 45 may be put, is for protecting telephone and like cables, which are laid beneath the street and which frequently become damp with sewer gas and ground moisture and 50 coated with frost. These cables are composed of hundreds of small wires. When these become damp, due to leaks in the lead sheathes of the cable, they have to be removed and each wire dried. The present composition may be injected, by a squirt gun,

into an opening made in the cable in the vicinity of the short, and all of the wires will be coated and insulated thereby.

The composition constituting the present invention consists of the following ingredients taken in the appended approximate proportions:—

|                    | Per cent |
|--------------------|----------|
| Boiled linseed oil | 52       |
| Japan dryer        | 26 60    |
| Olive oil          | 20       |
| Pumice stone       | 1        |
| Brown coloring oil | 1        |

The linseed oil in the composition oxidizes in the usual manner and forms a protecting 65 skin over the covered surface against moisture and other atmospheric conditions and the japan dryer supplements the oil and aids in its oxidation.

The olive oil prevents the linseed oil and 70 dryer from becoming too hard and brittle and keeps the same from cracking. In other words, it keeps the coating formed flexible. In addition, this oil operates as an insulator to maintain the temperature of the solution 75 and the covering formed thereby fairly constant at all times.

The pumice stone gives body and substance 80 to the mixture, makes it easier to apply and also acts as an insulator.

As previously stated, the purpose of the composition is to protect the coils, wires, plugs, distributor caps, and all other parts of any ignition system from dampness, moisture and any other atmospheric conditions. 85 If the ignition system, or any part thereof, is already wet, this solution will immediately prevent short circuits and prevent leakage of electric current from the ignition system.

It will also be readily apparent that the 90 composition may be readily applied to the wires and other parts of a system by means of a brush from which it will readily flow and form an even coating over the body to which it is applied. By employing the japan 95 dryer the composition will oxidize sufficiently rapidly to prevent its gravitating to the under side of the wire or other body on which it is placed, and dripping therefrom before it is set.

Having thus described my invention, what I claim is:—

1. An insulating composition of the character described having as the essential ingredients boiled linseed oil, japan dryer, olive oil, and pumice stone.
2. A composition for insulating electrical elements consisting of boiled linseed oil 52%, japan dryer 26%, olive oil 20%, pumice stone 10 1%, and a suitable coloring material constituting the remaining 1%.

In testimony whereof I hereunto affix my signature.

OLIVER B. HUSKEY.

15

20

25

30

35

40

45

50

55

60

65

25

50

65

60

65

70

65

70

65